# EUROPEAN PATENT SPECIFICATION

(11) **EP 3 517 632 B1**
(45) Date of publication and mention of the grant of the patent: **24.11.2021**
(21) Application number: 17879791.6
(22) Date of filing: 12.12.2017
(51) Int. Cl.: C22B 1/20, C21B 5/00, C21B 5/04, C22B 1/16

(54) **BLAST FURNACE OPERATION METHOD**
VERFAHREN ZUM BETRIEB EINES HOCHOFENS
PROCÉDÉ DE FONCTIONNEMENT D'UN HAUT-FOURNEAU

(30) Priority: 16.12.2016 JP 2016243989
(43) Date of publication of application: 31.07.2019
(73) Proprietor: JFE Steel Corporation, Tokyo 100-0011 (JP)
(72) Inventor: IWAMI Yuji, Tokyo 100-0011 (JP); NONAKA Shunsuke, Tokyo 100-0011 (JP); HAYASAKA Yasukazu, Tokyo 100-0011 (JP)
(74) Representative: Haseltine Lake Kempner LLP
(86) International application number: PCT/JP2017/044474
(87) International publication number: WO 2018/110521

(56) References cited:
- JP-A- S5 651 507
- JP-A- S5 751 206
- JP-A- H06 108 124
- JP-A- S60 262 926
- JP-A- 2001 107 115
- JP-A- 2008 240 109
- JP-A- 2011 038 735
- JP-A- 2013 147 718
- JP-A- 2016 130 341
- RU-C2- 2 240 351

## Description

### Technical Field

The present invention relates to a blast furnace operation method involving adjusting consumptions of blast furnace feed materials, and in particular, to a blast furnace operation method involving measuring component concentrations of sintered ore, which is a blast furnace feed material, and using the component concentrations to adjust consumptions of blast furnace feed materials.

### Background Art

Currently, in blast furnace ironmaking methods, iron-bearing materials such as sintered ore, lump iron ore and pellets are mainly used as iron sources for blast furnace feed materials. Sintered ore is a type of agglomerated ore and is obtained as follows. Iron ore having particle sizes less than or equal to 10 mm, miscellaneous iron sources, such as various types of dust generated in ironworks, CaO-bearing materials, such as limestone, quick lime, and slags, auxiliary materials serving as a SiO₂ source or a MgO source, such as silica stone, serpentinite, dolomite, and nickel refining slags, and a solid fuel (carbonaceous material) serving as a binding material, such as coke breeze and anthracite, are mixed together with the addition of water in a drum mixer to be granulated and then burned.

In recent years, the concentration of iron present in a sintering raw material, which is a raw material for sintered ore, has been decreasing, and instead, the component concentration of gangue, such as SiO₂ and Al₂O₃, has been increasing. The component concentrations of ores produced have become inconsistent to such an extent that, even in ores of the same type, the component concentrations may vary for each imported shipment.

Variations in the component concentrations of a sintering raw material lead to variations in the component concentrations of sintered ore, which is a product. In general, the component concentrations of a material that is charged into a blast furnace are consistently managed for the purpose of controlling the quality of slags, for example. If a component concentration increases, another component needs to be added as an auxiliary material to dilute the component concentration. It is, therefore, necessary to quickly detect a change in component concentrations of sintered ore, lump iron ore, and pellets. Lump iron ore and pellets are products themselves, and, therefore, analysis of component concentrations is performed when, for example, products are unloaded. With regard to sintered ore, however, no online analysis of component concentrations is currently performed, and the current situation is that analysis of component concentrations is very seldom performed.

If, as a result of a change in the component concentrations of sintered ore, the component concentrations of a blast furnace feed material change and significantly deviate from target component concentrations, and, consequently, the appropriate viscosity of slags deteriorates, it is necessary to increase the temperature of the molten iron to maintain the viscosity of slags. Deterioration in the viscosity of slags leads to deterioration in discharging of slags in a lower portion of a blast furnace, which interferes with the flow of gases and degrades gas permeability. As a result, for example, a need for increasing a consumption of coke to supplement the molten iron temperature and gas permeability may arise. Thus, when the component concentrations of a blast furnace feed material significantly deviate from target component concentrations, the operation of the blast furnace becomes unstable, and various countermeasures need to be taken.

Technologies for ascertaining the quality of sintered ore include the following, for example. Patent Literature 1 discloses a technology in which the reducibility and the reduction degradation property of product sintered ore are predicted from the sintering raw material filling status, and, a consumption of a sintering raw material, rather than a consumption ratio for blast furnace feed materials, is adjusted to adjust the blast furnace feed materials.

Patent Literature 2 discloses a technology in which FeO in product sintered ore is measured, and, on the basis of the difference from an aimed target value, the binding material for the sintering raw material, the water content for granulation, and the amount of exhaust air are adjusted. Furthermore, Patent Literature 3 discloses a technology in which, similarly, FeO in product sintered ore is measured, and, on the basis of the difference from an aimed target value, the amount of city gas to be injected into a sintering machine is adjusted.

Patent Literature 4 discloses a technology in which the components of product sintered ore are estimated on the basis of the components in a surface layer of a sintering raw material, which are determined by a laser-type component analyzer provided on a sintering machine, and, a sintering raw material is formulated in a manner that reflects the estimate.

PTL 5 discloses a blast furnace operation method wherein the chemical composition of raw materials to be charged into the blast furnace is measured with the lapse of time.

PTL 6 discloses a method of improving the chemical composition of slag in blast furnace smelting.

PTL 7 discloses a method of producing sintered ore raw material using magnetite ore.

PTL 8 discloses an operating method of a blast furnace.

### Citation List

### Patent Literature

PTL 1: Japanese Unexamined Patent Application Publication No. 10-324929
PTL 2: Japanese Unexamined Patent Application Publication No. 57-149433
PTL 3: Japanese Unexamined Patent Application Publication No. 2011-038735
PTL 4: Japanese Unexamined Patent Application Publication No. 60-262926
PTL 5: Japanese Unexamined Patent Application Publication No. S57-51206
PTL 6: Russian Patent No. 2240351 C2
PTL 7: JP 2016 130341 A
PTL 8: JP S56 51507 A

### Summary of Invention

### Technical Problem

The technologies disclosed in Patent Literature 1 to Patent Literature 4, however, are technologies in which a particular component concentration of sintered ore is measured and, by using the measured component concentration, the sintering raw material is adjusted or the conditions for producing sintered ore are adjusted. None of Patent Literature 1 to Patent Literature 4 discloses adjusting, by using a measured component concentration of sintered ore, the consumptions of blast furnace feed materials to be charged into a blast furnace. Since the component concentrations of sintered ore can also change with the heat level during the sintering reaction, inhibiting changes in the component concentrations of a sintering raw material does not necessarily inhibit changes in the component concentrations of sintered ore. Thus, there has been a problem in that the component concentrations of blast furnace feed materials to be charged into a blast furnace cannot be controlled to target component concentrations. The present invention was made in view of such problems of the related art, and an object of the present invention is to provide a blast furnace operation method that makes it possible to control the component concentrations of blast furnace feed materials to target component concentrations even if there is a change in the component concentrations of a sintering raw material.

### Solution to Problem

The present invention solves the above problems through a method according to claim 1. Further advantageous embodiments of the method are described in dependant claims 2-5.

### Advantageous Effects of Invention

By implementing the blast furnace operation method of the present invention, the component concentrations of blast furnace feed materials can be controlled to target component concentrations. Consequently, changes in the viscosity of blast furnace slags, for example, are inhibited, which contributes to stable operation of a blast furnace.

### Brief Description of Drawings

[Fig. 1] Fig. 1 is a schematic diagram illustrating an example of a sintered ore production apparatus 10, which can implement a blast furnace operation method according to the present embodiment.
[Fig. 2] Fig. 2 is a graph illustrating changes in the basicity of blast furnace slags.
[Fig. 3] Fig. 3 is a graph illustrating changes in the coke ratio.
[Fig. 4] Fig. 4 is a graph illustrating changes in the basicity of blast furnace feed materials and changes in the coke ratio.
[Fig. 5] Fig. 5 is a graph illustrating measured values of FeO concentrations of Invention Example 3, Invention Example 4, and Comparative Example 3.
[Fig. 6] Fig. 6 is a graph illustrating amounts of reduction in the coke ratio of Invention Example 3, Invention Example 4, and Comparative Example 3. Description of Embodiments

In the present invention, a measuring step for measuring component concentrations of sintered ore is provided, and component concentrations of sintered ore are measured in the measuring step. By using the component concentrations measured, the consumptions of product sintered ore, pellets, lump iron ore, and an auxiliary material, which are blast furnace feed materials, are adjusted. Consequently, the component concentrations of blast furnace feed materials can be controlled to reach target component concentrations, and as a result, stable blast furnace operation is made possible. With this finding, the present invention was made. The present invention will now be described with reference to an embodiment of the present invention.

Fig. 1 is a schematic diagram illustrating an example of a sintered ore production apparatus 10, which can implement a blast furnace operation method according to the present embodiment. A sintered ore production apparatus 10 includes a sintering machine 12, a primary crusher 14, a cooler 16, a secondary crusher 18, a plurality of sieving devices 20, 22, 24, 26, an infrared analyzer 28, a product line 30, and a return ore line 32.

The sintering machine 12 performs a sintering step. The sintering machine 12 is, for example, a downward-suction-type Dwight-Lloyd sintering machine. The sintering machine 12 includes a sintering raw material feeding device, an endless-moving-type pallet, an ignition furnace, and wind boxes. A sintering raw material is charged into the pallet through the sintering raw material feeding device, thereby forming a burden layer of the sintering raw material. The ignition furnace ignites the burden layer. Air within the burden layer is sucked downwardly through the wind boxes, thereby moving the combustion and melting zone within the burden layer toward a lower portion in the burden layer. In this manner, the burden layer is sintered to form a sintered cake. When air within the burden layer is sucked downwardly through the wind boxes, a gas fuel and/or oxygen-gas-enriched air may be supplied from above the burden layer. The gas fuel is a combustible gas selected from the following: blast furnace gas, coke oven gas, a mixed gas of a blast furnace gas and coke oven gas, converter gas, city gas, natural gas, methane gas, ethane gas, propane gas, and a mixed gas thereof.

The primary crusher 14 performs a crushing step. A sintered cake is crushed by the primary crusher 14 to form sintered ore. The cooler 16 performs a cooling step. Sintered ore is cooled by the cooler 16 to form cooled sintered ore.

The sieving devices 20, 22, 24, 26 perform a sieving step. By using the sieving device 20, cooled sintered ore is sieved and separated into sintered ore having particle sizes greater than 75 mm and sintered ore having particle sizes less than or equal to 75 mm. In the present embodiment, "particle sizes" refers to particle sizes determined by performing sieving with a sieve: for example, "sintered ore having particle sizes greater than 75 mm" refers to particle sizes such that sintered ore, when sieved with a sieve having an opening size of 75 mm, is retained on the sieve, and "sintered ore having particle sizes less than or equal to 75 mm" refers to particle sizes such that sintered ore, when sieved with a sieve having an opening size of 75 mm, is not retained on the sieve.

Sintered ore having particle sizes greater than 75 mm, which is retained on the sieve when sieved with the sieving device 20, is crushed with the secondary crusher 18 to reduce the particle sizes to less than or equal to 50 mm. The crushed sintered ore is mixed with non-retained sintered ore, and the mixture is sieved with the sieving device 22. This ensures that the upper limit of the particle sizes of product sintered ore is not greater than 75 mm.

Sintered ore having particle sizes less than or equal to 75 mm, which is not retained on the sieve when sieved with the sieving device 20, is subsequently sieved and separated, by using the sieving devices 22, 24, 26, into product sintered ore having particle sizes greater than 5 mm and return ore having particle sizes less than or equal to 5 mm. Product sintered ore, which is sieved and separated with the sieving devices 22, 24 and 26, is transferred to a blast furnace 34 by a conveyor belt that forms the product line 30. On the other hand, return ore, which is sieved and separated with the sieving devices 22, 24 and 26, is transferred to the sintering raw material feeding device of the sintering machine 12 again by a conveyor belt that forms the return ore line 32. The value of the particle sizes of sintered ore that is sieved and separated using the sieving devices 20, 22, 24, 26, the value of the particle sizes of product sintered ore, and the value of the particle sizes of return ore are merely examples, and therefore the values are non-limiting.

The conveyor belt that forms the product line 30 is provided with the infrared analyzer 28. The infrared analyzer 28 performs the measuring step. In the measuring step, the component concentration of at least one of total CaO, SiO₂, MgO, Al₂O₃, and FeO that are present in product sintered ore are measured. The infrared analyzer 28 radiates infrared light having wavelengths ranging from 0.5 µm to 50.0 µm onto sintered ore and receives reflected light from the sintered ore. Total CaO, SiO₂, MgO, Al₂O₃, and FeO that are present in sintered ore each have molecular vibrations and each absorb a specific-wavelength component of the radiated infrared light, and therefore each of the components imparts a specific-wavelength component to reflected infrared light. Accordingly, the component concentrations of total CaO, SiO₂, MgO, Al₂O₃, and FeO in product sintered ore can be measured by analyzing the radiated light and the reflected light. Total CaO is determined by calculating Ca in all compounds including Ca and O, such as CaO, CaCO₃, Ca(OH)₂, and Fe₂CaO₄, as CaO.

For example, the infrared analyzer 28 radiates infrared light having 20 or more wavelengths and receives reflected light reflected from sintered ore, at a frequency of 128 times per minute. By radiating infrared light in a short time as described above, the infrared analyzer 28 can measure, on-line and sequentially, the component concentrations of sintered ore, which is transferred on the conveyor belt that forms the product line 30. The infrared analyzer 28 is an example of a component analysis instrument. The component analysis instrument is not limited to an instrument of the type that spectrally analyzes reflected light and may be an instrument of the type that spectrally analyzes transmitted light. In place of the infrared analyzer 28, it is possible to use a laser analyzer that radiates laser beams onto an object to be measured, a neutron analyzer that radiates neutrons onto an object to be measured, or a microwave analyzer that radiates microwaves onto an object to be measured.

After the component concentrations of product sintered ore is measured, the product sintered ore is transferred to the blast furnace 34, and is subjected to an adjusting step in which the consumptions of blast furnace feed materials including product sintered ore, pellets, lump iron ore, and an auxiliary material are adjusted. The blast furnace feed materials may include one or more other materials in addition to the materials mentioned above or may not include pellets. In the adjusting step, the total component amounts of the blast furnace feed materials are calculated by using the component concentrations of the product sintered ore measured using the infrared analyzer 28 and premeasured component concentrations of pellets, lump iron ore, and an auxiliary material, and, by using the calculated value, feed-forward control is performed on the consumptions of the blast furnace feed materials to obtain target component concentrations. For example, the basicity (CaO/SiO₂) of the blast furnace feed materials can be controlled to target component concentrations by adjusting the consumption of an auxiliary material to be included in the blast furnace feed materials.

If the FeO concentration of product sintered ore is high, and, consequently, the FeO concentration of blast furnace feed materials is high, the reducibility of the blast furnace feed materials deteriorates. When the reducibility of blast furnace feed materials deteriorates, indirect reduction, which is an exothermic reaction, decreases, and direct reduction, which is an endothermic reaction, increases, and as a result, the heat within the blast furnace becomes insufficient. To resolve the heat insufficiency, an additional amount of reducing agent has to be charged into the blast furnace, which results in an increase in the coke ratio for blast furnace operation. Accordingly, by controlling the FeO concentration of blast furnace feed materials to a target component concentration, an increase in the coke ratio for blast furnace operation can be inhibited, which contributes to stable blast furnace operation. For example, FeO in blast furnace feed materials can be controlled to a target component concentration by adjusting the consumption of lump ore to be included in the blast furnace feed materials.

As described above, the consumptions of blast furnace feed materials are adjusted to ensure that the component concentrations of the blast furnace feed materials correspond to target component concentrations. In the present embodiment, the frequency at which component concentrations are measured using the infrared analyzer 28 is 128 times per minute, and the average of the 128 component concentrations was calculated once per minute, and, by using the calculated average of the component concentrations, the consumptions of the blast furnace feed materials were adjusted every minute.

As described above, in the blast furnace operation method according to the present embodiment, component concentrations of product sintered ore, which is transferred on the product line 30, are measured using the infrared analyzer 28, and, by using the measured component concentrations, the consumptions of the blast furnace feed materials are adjusted to ensure that target component concentrations are obtained. As a result, even if the component concentrations of a sintering raw material change and consequently the component concentrations of product sintered ore change, the component concentrations of blast furnace feed materials can be controlled to target component concentrations. Charging such blast furnace feed materials into a blast furnace results in stable blast furnace operation and inhibits an increase in the coke ratio for blast furnace operation.

In the example described in the present embodiment, the infrared analyzer 28 is provided at the conveyor belt that forms the product line 30, and, component concentrations of product sintered ore are measured. However, this example is non-limiting. The infrared analyzer 28 may be provided at any of one or more locations of the sintered ore production apparatus 10, and component concentrations of at least one or more of cooled sintered ore, product sintered ore, and return ore may be measured.

In a burden layer, which is formed of a sintering raw material charged into a pallet, the component concentrations significantly differ between a surface layer and a lower layer, and, the component concentrations change with the water content of a sintering raw material and/or the condition of a sintering raw material feeding device. Because of its nature, analysis using infrared light is only capable of analyzing a surface layer of an object to be analyzed. Thus, even when the burden layer, in which the component concentrations differ between a surface layer and a lower layer and so the component concentrations change, is measured with the infrared analyzer 28, the component concentrations of the entire burden layer cannot be measured with high precision. In contrast, after the cooling step, with the sintering raw material having been sintered, crushed, cooled, and homogenized to some extent, the component concentrations of a surface layer and the component concentrations of a lower layer are not significantly different from each other. For this reason, in the measuring step of the present embodiment, component concentrations of at least one of post-cooling-step sintered ore, product sintered ore, and return ore are measured. As a result, even with an infrared analyzer 28 that is only capable of analyzing a surface layer of an object to be analyzed, component concentrations can be measured with high precision.

When the particle size distribution of sintered ore is broad, infrared light can be radiated only onto a portion of the sintered ore because, for example, infrared light cannot be radiated onto sintered ore having small particle sizes that is hidden behind sintered ore having large particle sizes, and furthermore, reflected light from sintered ore is unstable. In contrast, after the sieving step, with the sintered ore having been sieved and separated into product sintered ore having particle sizes greater than 5 mm and return ore having particle sizes less than or equal to 5 mm, the particle size distribution of sintered ore is narrow. For this reason, it is preferable that component concentrations of at least one of product sintered ore and return ore, which are post-sieving-step ores, be measured in the measuring step. Accordingly, the infrared analyzer 28 can radiate infrared light onto sintered ore uniformly, and reflected light from sintered ore is stable. As a result, component concentrations can be measured with higher precision.

Thus, after the sieving step, component concentrations of product sintered ore or return ore may be measured in the measuring step, but it is more preferable to measure product sintered ore rather than return ore because component concentrations of product sintered ore, which is used as one of the blast furnace feed materials, can be directly measured.

### EXAMPLE 1

The component concentrations of total CaO, SiO₂, MgO, Al₂O₃, and FeO that are present in product sintered ore were measured at a frequency of once per minute by using a sintered ore production apparatus 10, in which an infrared analyzer 28 was provided at a product line 30. Invention Example 1 is an operation example in which the consumption of an auxiliary material of blast furnace feed materials was adjusted at a frequency of once per minute by using the measurement results. Comparative Example 1 is an operation example in which the consumption of an auxiliary material of blast furnace feed materials was not adjusted. The blast furnace coke ratio and changes in the basicity of blast furnace slags in Comparative Example 1 and Invention Example 1 were measured.

Fig. 2 is a graph illustrating changes in the basicity of blast furnace slags. Fig. 2(a) illustrates changes in the basicity of Comparative Example 1, and Fig. 2(b) illustrates changes in the basicity of Invention Example 1. In Fig. 2, the horizontal axis represents time (day), and the vertical axis represents total CaO/SiO₂ (-). The values of the basicity shown in Fig. 2 are values determined by performing chemical analysis off-line on the components of molten iron and blast furnace slags tapped from the blast furnace.

In Comparative Example 1, the basicity significantly varied around the target value, as illustrated in Fig. 2. In contrast, in Invention Example 1, deviations of the basicity from the target value were small because component concentrations of product sintered ore were measured at a frequency of once per minute, and, by using the component concentrations, the consumption of blast furnace feed materials was adjusted to ensure that the component concentrations of the blast furnace feed materials would correspond to target component concentrations. Thus, it was verified that, by implementing the blast furnace operation method according to the present embodiment, deviations of the basicity of blast furnace slags from a target value can be reduced.

Fig. 3 is a graph illustrating changes in the coke ratio. In Fig. 3, the horizontal axis represents time (day), and the vertical axis represents coke ratios (kg/t-pig). The coke ratios of 0th day to 19th day are coke ratios of Comparative Example 1, in which blast furnace operation was performed by charging blast furnace feed materials for which no adjustment of the consumptions was made. The coke ratios of 20th day to 39th day are coke ratios of Invention Example 1, in which blast furnace operation was performed by charging blast furnace feed materials for which adjustment of a consumption was made at a frequency of once per minute.

As illustrated in Fig. 3, the coke ratio in blast furnace operation was lower in Invention Example 1 than in Comparative Example 1. Thus, it was verified that, by implementing the blast furnace operation method according to the present embodiment, blast furnace operation can be stabilized, and as a result, the coke ratio for blast furnace operation can be inhibited from increasing.

### EXAMPLE 2

Fig. 4 is a graph illustrating changes in the basicity of blast furnace feed materials and changes in the coke ratio. Fig. 4(a) illustrates changes in the basicities of blast furnace feed materials of Comparative Example 2 and Invention Example 2. In Fig. 4(a), the horizontal axis represents time (hour), and the vertical axis represents total CaO/SiO₂ (-) of blast furnace feed materials. Fig. 4(b) illustrates changes in the coke ratios for blast furnace operation of Comparative Example 2 and Invention Example 2. In Fig. 4(b), the horizontal axis represents time (hour), and the vertical axis represents coke ratios (kg/t-pig).

In Fig. 4, Comparative Example 2 is an operation example in which total CaO and SiO₂ in product sintered ore were measured at a frequency of once every two hours by using X-ray fluorescence, and, by using the measurement results, the consumption of an auxiliary material of blast furnace feed materials was adjusted at the same frequency. Invention Example 2 is an operation example in which, similarly to Invention Example 1, the component concentrations of total CaO and SiO₂ in product sintered ore were determined at a frequency of once per minute by using the infrared analyzer 28 provided at the production line 30, and, by using the measurement results, the consumption of an auxiliary material of blast furnace feed materials was adjusted at the same frequency.

In the examples illustrated in Fig. 4, blast furnace operation was performed under the conditions of Comparative Example 2 from 0th hour to 6th hour, and blast furnace operation was performed under the conditions of Invention Example 2 from 6th hour to 19th hour. As illustrated in Fig. 4(a), in Comparative Example 2, too, the consumption of an auxiliary material was adjusted at a frequency of once every two hours, and therefore, changes in the basicity of the blast furnace feed materials appeared to be inhibited in a measurement performed once every two hours. However, when Comparative Example 2 was replaced with Invention Example 2 and the consumption of an auxiliary material of blast furnace feed materials was adjusted at a frequency of once per minute, the coke ratio for blast furnace operation, as illustrated in Fig. 4(b), began to decrease at or around the time at which, presumably, blast furnace feed materials in which the consumption was adjusted was charged into the blast furnace. In general, sintered ore discharged from a sintering machine is cooled with a cooler and subjected to sizing and is thereafter charged, by way of an ore bin of a blast furnace, into the blast furnace. Although depending on the size of an ore bin, the residence time for materials in the ore bin used in this example was approximately eight hours, and therefore it can be considered that the effect began to gradually show in the blast furnace after eight hours.

Thus, in the measurement performed once every two hours, changes in the basicity appeared to be inhibited, but presumably, the basicity of the blast furnace feed materials changed in the intermediate periods, and under this influence, the coke ratio of Comparative Example 2 increased. In contrast, in Invention Example 2, the infrared analyzer 28 was provided at the product line 30, the measurement of total CaO and SiO₂ in product sintered ore was performed at a frequency of once per minute, and, by using the measurement results, the consumption of an auxiliary material was adjusted to ensure that the basicity of the blast furnace feed materials would correspond to a target value, and therefore, presumably, changes in the basicity of the blast furnace feed materials were inhibited even in the intermediate period within two hours, and as a result, the coke ratio for blast furnace operation was inhibited from increasing.

### EXAMPLE 3

Fig. 5 is a graph illustrating measured values of FeO concentrations of Invention Example 3, Invention Example 4, and Comparative Example 3. In Fig. 5, the vertical axis represents measured values (mass%) of the FeO concentration at a specific time.

Invention Example 3 is an operation example in which the infrared analyzer 28 was provided at the production line 30, the component concentrations of total CaO, SiO₂, MgO, Al₂O₃, and FeO in product sintered ore were measured at a frequency of once per minute, and, by using the measurement results, the consumption of an auxiliary material of blast furnace feed materials was adjusted at a frequency of once per minute. Invention Example 4 is an operation example in which the infrared analyzer 28 was provided at a return ore line 32, the component concentrations of total CaO, SiO₂, MgO, Al₂O₃, and FeO in product sintered ore were measured at a frequency of once per minute, and, by using the measurement results, the consumption of an auxiliary material of blast furnace feed materials was adjusted at a frequency of once per minute. Comparative Example 3 is an operation example in which the infrared analyzer 28 was provided at a location of a sintering machine 12 where measurement of the surface of a sintered cake was able to be performed, the component concentrations of total CaO, SiO₂, MgO, Al₂O₃, and FeO in the surface of the sintered cake were measured at a frequency of once per minute, and, by using the measurement results, the consumption of an auxiliary material of blast furnace feed materials was adjusted at a frequency of once per minute.

As illustrated in Fig. 5, a FeO concentration determined by measuring product sintered ore was 7.1 mass%, whereas a FeO concentration determined by measuring return ore produced from the same sintering raw material was 6.9 mass%. This result indicates that the result of measurement of the FeO concentration of return ore and the result of measurement of the FeO concentration of product sintered ore, which were performed by using the infrared analyzer, were not significantly different from each other. In contrast, a FeO concentration determined by measuring, by using the infrared analyzer 28, the surface of a sintered cake obtained by sintering the same sintering raw material was 5.6 mass%, which was significantly different from the FeO concentration determined by measuring product sintered ore.

Because of its nature, an infrared analyzer is only capable of measuring component concentrations in the surface irradiated with infrared light. By radiating infrared light onto the surface of product sintered ore or return ore, average components of the entirety can be determined. This is because product sintered ore or return ore either is homogenized to some extent in the process of crushing. On the other hand, in a sintered cake, a significant difference is generated between the component concentrations of an upper layer and those of a lower layer. This is because the component concentrations of a sintering raw material charged into the pallet differ between an upper layer and a lower layer, and, the heat level during sintering differs between an upper layer and a lower layer. It is presumed that, for the above reasons, the component concentrations of Comparative Example 3, in which the surface of a sintered cake was measured with the infrared analyzer, were significantly different from the component concentrations of Invention Example 3, in which the surface of product sintered ore was measured, as illustrated in Fig. 5.

Fig. 6 is a graph illustrating amounts of reduction in the coke ratio of Invention Example 3, Invention Example 4, and Comparative Example 3. In Fig. 6, the vertical axis represents amounts of reduction in the coke ratio (kg/t-pig). The amount of reduction in the coke ratio illustrated in Fig. 6 is an amount of reduction determined using a coke ratio obtained before adjusting the consumptions of the blast furnace feed materials and a coke ratio obtained when, supposedly, the influence of operation variations had diminished and the operation had entered a steady state, after 120 hours elapsed from the time at which the consumptions of the blast furnace feed materials were adjusted in accordance with Invention Example 3, Invention Example 4, or Comparative Example 3.

In Invention Example 3, in which the consumption of an auxiliary material of the blast furnace feed materials was adjusted by using component concentrations of product sintered ore to be charged into the blast furnace as a blast furnace feed material, and in Invention Example 4, in which the consumption of an auxiliary material of the blast furnace feed materials was adjusted by using component concentrations of return ore having component concentrations similar to the component concentrations of product sintered ore, the coke ratio at a point in time after 120 hours elapsed was reduced. On the other hand, in Comparative Example 3, in which the consumption of an auxiliary material of the blast furnace feed materials was adjusted by using a measured value of a sintered cake, which had component concentrations significantly different from those of product sintered ore to be charged into the blast furnace, the coke ratio at a point in time after 120 hours elapsed, on the contrary, was increased. It is presumed that this was a result attributable to the fact that, in Comparative Example 3, the component concentrations of the blast furnace feed materials to be charged into the blast furnace were not adjusted to target component concentrations.

### Reference Signs List

- 10: Sintered ore production apparatus
- 12: Sintering machine
- 14: Primary crusher
- 16: Cooler
- 18: Secondary crusher
- 20: Sieving device
- 22: Sieving device
- 24: Sieving device
- 26: Sieving device
- 28: Infrared analyzer
- 30: Product line
- 32: Return ore line
- 34: Blast furnace

## Claims

1. A blast furnace operation method including charging blast furnace feed materials into a blast furnace (34), the blast furnace feed materials including product sintered ore, lump iron ore, and an auxiliary material for control of the slag basicity defined by CaO/SiO₂, the blast furnace operation method comprising:
a sintering step for sintering a sintering raw material to form a sintered cake;
a crushing step for crushing the sintered cake to form sintered ore;
a cooling step for cooling the sintered ore;
a sieving step for sieving the cooled sintered ore to separate into product sintered ore and return ore;
a measuring step for measuring a component concentration of at least one of the cooled sintered ore, the product sintered ore, and the return ore, each being transferred on a conveyor (30,32), by using an infrared analyzer (28), or a laser analyzer, or a neutron analyzer or a microwave analyzer; and
an adjusting step for adjusting consumptions of the product sintered ore, the lump iron ore, and the auxiliary material, which are to be included in the blast furnace feed materials,
wherein, in the adjusting step, the total component amounts of the blast furnace feed materials are calculated by using the component concentrations of at least one of the cool sintered ore, the product sintered ore and the return ore measured in the measuring step and premeasured component concentrations of lump iron ore, and the auxiliary material, and by using the calculated value, feed forward control is performed by adjusting the consumptions of the blast furnace feed materials by using the component concentration measured in the measuring step.

2. The blast furnace operation method according to Claim 1, wherein,
the blast furnace feed materials further include pellets, and
in the adjusting step, consumptions of the product sintered ore, the pellets, the lump iron ore, and the auxiliary material, which are to be included in the blast furnace feed materials, are adjusted.

3. The blast furnace operation method according to Claim 1 or 2, wherein, in the measuring step, the component concentration of at least one of the product sintered ore and the return ore is measured.

4. The blast furnace operation method according to Claim 1 or 2, wherein, in the measuring step, the component concentration of the product sintered ore is measured.

5. The blast furnace operation method according to any one of Claims 1 to 4, wherein, in the measuring step, a component concentration of at least one of total CaO, SiO₂, MgO, Al₂O₃, and FeO is measured.

## Patentansprüche

1. Hochofen-Betriebsverfahren, das die Beschickung eines Hochofens (34) mit Hochofeneinsatzmaterial umfasst, wobei die Hochofen-Einsatzmaterialien das Produkt gesintertes Erz, stückiges Eisenerz und einen Hilfsstoff zur Kontrolle der durch CaO/SiO₂ definierten Schlackenbasizität umfassen, wobei das Hochofen-Betriebsverfahren umfasst:
einen Sinterschritt zum Sintern eines Sinter-Rohmaterials, um einen Sinterkuchen zu bilden;
einen Zerkleinerungsschritt zum Zerkleinern des Sinterkuchens, um gesintertes Erz zu bilden;
einen Kühlschritt zum Kühlen des gesinterten Erzes;
einen Siebschritt zum Sieben des gekühlten gesinterten Erzes, um in das Produkt Sintererz und Rücklauferz zu trennen;
einen Messschritt zum Messen der Konzentration einer Komponente von mindestens einem Element aus dem gekühlten Sintererz, dem Produkt Sintererz und dem Rücklauferz, wobei jedes auf einem Förderband (30, 32) transportiert wird, wobei ein Infrarot-Analysator (28) oder ein Laser-Analysator oder ein Neutronen-Analysator oder ein Mikrowellen-Analysator verwendet wird, und
einen Einstellschritt zum Einstellen der Verbrauchsdaten des Produktes gesintertes Erz, des stückigen Eisenerzes und des Hilfsstoffs, die zu den Hochofen-Einsatzmaterialien gehören,
wobei im Einstellschritt die Gesamtmengen der Komponenten der Hochofen-Einsatzmaterialien unter Verwendung der Komponentenkonzentrationen von mindestens einer Komponente aus dem gekühlten Sintererz, dem Produkt Sintererz und dem Rücklauferz, die im Messschritt gemessen wurden, und vorgemessene Komponentenkonzentrationen von stückigem Eisenerz und dem Hilfsstoff berechnet werden, und unter Verwendung des berechneten Wertes wird eine Optimalwertsteuerung durch Einstellen der Verbrauchsdaten der Hochofen-Einsatzmaterialien mittels der Komponentenkonzentration, die im Messschritt gemessen wurde, vorgenommen.

2. Hochofen-Betriebsverfahren nach Anspruch 1, wobei
die Hochofen-Einsatzmaterialien ferner Pellets enthalten, und
im Einstellschritt die Verbrauchsdaten des Produktes Sintererz, der Pellets, des stückigen Eisenerzes und des Hilfsstoffs, die zu den Hochofen-Einsatzmaterialien gehören, eingestellt werden.

3. Hochofen-Betriebsverfahren nach Anspruch 1 oder 2, wobei im Messschritt die Komponentenkonzentration von mindestens einem Element aus dem Produkt Sintererz und dem Rücklauferz gemessen wird.

4. Hochofen-Betriebsverfahren nach Anspruch 1 oder 2, wobei im Messschritt die Komponentenkonzentration des Produktes Sintererz gemessen wird.

5. Hochofen-Betriebsverfahren nach Anspruch 1 bis 4, wobei im Messschritt die Komponentenkonzentration von mindestens einem Element aus dem gesamten CaO, SiO₂, MgO, Al₂O₃ und FeO gemessen wird.

## Revendications

1. Procédé d'exploitation de haut fourneau comprenant un chargement de matières d'alimentation de haut fourneau dans un haut fourneau (34), les matières d'alimentation de haut fourneau comprenant du minerai fritté produit, du minerai de fer en morceaux et une matière première auxiliaire pour une commande de la basicité du laitier définie par CaO/SiO₂, le procédé de fonctionnement de haut fourneau comprenant :
une étape de frittage pour fritter une matière première de frittage pour former un gâteau fritté ;
une étape de broyage pour broyer le gâteau fritté afin de former du minerai fritté ;
une étape de refroidissement pour refroidir le minerai fritté ;
une étape de tamisage pour tamiser le minerai fritté refroidi afin de le séparer en minerai fritté produit et en minerai de retour ;
une étape de mesure pour mesurer une concentration de composant d'au moins un parmi le minerai fritté refroidi, le minerai fritté produit, et le minerai de retour, chacun étant transféré sur un convoyeur (30, 32), en utilisant un analyseur infrarouge (28), ou un analyseur laser, ou un analyseur neutronique ou un analyseur de micro-ondes ; et
une étape d'ajustement pour ajuster des consommations du minerai fritté produit, du minerai de fer en morceaux et de la matière première auxiliaire, qui doivent être inclus dans les matières d'alimentation de haut fourneau,
dans lequel, dans l'étape d'ajustement, les quantités de composant totales des matières d'alimentation de haut fourneau sont calculées en utilisant les concentrations de composant d'au moins un parmi le minerai fritté froid, le minerai fritté produit et le minerai de retour mesurées dans l'étape de mesure et des concentrations de composant mesurées préalablement du minerai de fer en morceaux, et de la matière auxiliaire, et en utilisant la valeur calculée, une commande d'avance d'alimentation est effectuée en ajustant les consommations des matières d'alimentation de haut fourneau en utilisant la concentration de composant mesurée dans l'étape de mesure.

2. Procédé d'exploitation de haut fourneau selon la revendication 1, dans lequel,
les matières d'exploitation de haut fourneau comprennent en outre des pastilles, et
dans l'étape d'ajustement, les consommations du minerai fritté produit, des pastilles, du minerai de fer en morceaux et de la matière auxiliaire, qui doivent être inclus dans les matières d'alimentation du haut fourneau, sont ajustées.

3. Procédé d'exploitation de haut fourneau selon la revendication 1 ou 2, dans lequel, dans l'étape de mesure, la concentration de composant d'au moins l'un du minerai fritté produit et du minerai de retour est mesurée.

4. Procédé d'exploitation de haut fourneau selon la revendication 1 ou 2, dans lequel, dans l'étape de mesure, la concentration de composant du minerai fritté produit est mesurée.

5. Procédé d'exploitation de haut fourneau selon l'une quelconque des revendications 1 à 4, dans lequel, dans l'étape de mesure, une concentration de composant d'au moins un parmi le CaO total, le SiO₂, le MgO, l'Al₂O₃ et le FeO est mesurée.
